

## [54] SPECTRALLY SENSITIZED SILVER HALIDE PHOTOGRAPHIC EMULSION

[75] Inventors: Keisuke Shiba; Haruo Takei; Akira Sato; Tadashi Ikeda, all of Kanagawa, Japan

[73] Assignee: Fuji Photo Film Co., Ltd., Kanagawa, Japan

[22] Filed: Sept. 24, 1971

[21] Appl. No.: 183,492

## [30] Foreign Application Priority Data

Sept. 24, 1970 Japan..... 45/83653

[52] U.S. Cl..... 96/124, 96/137

[51] Int. Cl..... G03c 1/14

[58] Field of Search..... 96/124, 137

## [56] References Cited

## UNITED STATES PATENTS

|           |        |                 |              |
|-----------|--------|-----------------|--------------|
| 2,066,966 | 1/1937 | Dieterle et al. | ..... 96/137 |
| 2,066,967 | 1/1937 | Dieterle et al. | ..... 96/137 |
| 3,679,428 | 7/1972 | Shiba et al.    | ..... 96/124 |

Primary Examiner—J. Travis Brown  
Attorney—Richard C. Sughrue et al.

## [57]

## ABSTRACT

A silver halide photographic emulsion containing a supersensitizing combination of at least one carbocyanine dye having a heterocyclic nucleus comprising a benzothiazole or benzoselenazole nucleus, at least one of the heterocyclic nuclei having an acetylarnino group at the 5-position thereof, and having a sensitized maximum portion within the range of from 600 to 660 nm, and at least one sensitizing dye of the following general formula (II)



wherein R<sub>3</sub> and R<sub>4</sub> each represents a lower alkyl group; A<sub>2</sub> represents a lower alkyl group or an aryl group; Z<sub>3</sub> and Z<sub>4</sub> each represents an atomic group necessary to complete a benzothiazole, benzoselenazole or β-naphthothiazole nucleus; X<sub>2</sub><sup>-</sup> represents an anion; and m is 0 or 1, m being 0 when an intermolecular salt is formed.

5 Claims, 4 Drawing Figures

PATENTED NOV 6 1973

3,770,449

**FIG. 1**



**FIG. 2**



**FIG. 3**



**FIG. 4**



# SPECTRALLY SENSITIZED SILVER HALIDE PHOTOGRAPHIC EMULSION

## BACKGROUND OF THE INVENTION

## 1. Field of the Invention

This invention relates to a spectrally sensitized silver halide photographic emulsion and more especially to a silver halide photographic emulsion which is supersensitized by the combined use of at least two sensitizing dyes resulting in a high red sensitivity.

## 2. Description of the Prior art

Photographic light sensitive materials which are used conventionally are required to have spectral sensitivity distributions corresponding to the photographing purpose.

In the manufacture of the sensitive material, it is an important technique to develop the combination of sensitizing dyes which are in supersensitization relation to each other and have a small inherent desensitization, i.e., a less desensitization, in the wavelength region inherent to silver halide grains.

The object of this invention is to provide a silver halide photographic emulsion having a panchromatically sensitized region, particularly a high red sensitivity within the spectro sensitized wavelength region of 640-685 nm and a small inherent desensitization by the combined use of two different types of sensitizing dyes.

A panchromatically sensitized region is used generally for black and white photographic sensitive materials.

## **SUMMARY OF THE INVENTION**

The object of this invention has been accomplished by the combined use of a carbocyanine dye comprising heterocyclic nuclei selected from benzothiazole and benzoselenazole nuclei, at least one of the heterocyclic nuclei having an acetylamino group at the 5-position thereof, and having a sensitized maximum portion within the range of from 600 to 660 nm., preferably of the following general formula (I), and a sensitizing dye of the general formula (II) in a silver halide photographic emulsion:



wherein  $R_1$  and  $R_2$  each represents a lower alkyl group, e.g., methyl, ethyl,  $\gamma$ -sulfopropyl,  $\gamma$ -sulfonybutyl,  $\delta$ -sulfobutyl, allyl etc.;  $A_1$  represents a lower alkyl group, e.g., methyl, ethyl etc.;  $Z_1$  represents an atomic group necessary to complete a benzothiazole or benzoselenazole nucleus, which may be substituted by a halogen atom, e.g., chlorine, etc., a lower alkyl group, e.g., methyl, ethyl, etc.; an alkoxy group, e.g., methoxy, ethoxy, etc.; or a phenyl group;  $Z_2$  represents a sulfur or selenium atom;  $X_1^-$  represents an anion, e.g., a chloride, bromide, iodide, perchlorate, p-toluene sulfonate, benzene sulfonate, thiocyanate, methyl sulfate or ethyl sulfate ion, etc.;  $n$  is 0 or 1 and  $n = 0$  for the intermolecular salt;



wherein  $R_3$  and  $R_4$  each represents lower alkyl, e.g. methyl, ethyl,  $\gamma$ -sulfopropyl,  $\gamma$ -sulfobutyl,  $\delta$ -sulfobutyl,  $\beta$ -hydroxyalkyl,  $\beta$ -carboxyalkyl, etc.;  $A_2$  represents lower alkyl, e.g. methyl, ethyl, etc., or an aryl group, e.g. phenyl;  $Z_3$  and  $Z_4$  each represents an atomic group necessary to complete a benzothiazole, benzoselenazole or  $\beta$ -naphthothiazole nucleus, which may be substituted by a halogen, e.g. chlorine or bromine, etc., a lower alkyl group, e.g. methyl, ethyl, etc.; alkoxy, e.g. methoxy, ethoxy etc.; a hydroxyl group or a phenyl group;  $X_2^-$  represents an anion, e.g., a chloride, bromide, iodide, p-toluene sulfonate or benzenesulfonate ion, etc. and those used generally in the art;  $m$  is 0 or 1 and  $m=0$  for the intermolecular salt.

#### BRIEF DESCRIPTION OF THE DRAWINGS

FIGS. 1-4 are spectrograms illustrating the supersensitization effects of the combination of dyes according to the present invention.

## DESCRIPTION OF THE PREFERRED EMBODIMENTS

Many cyanine dyes of the general formula (II) have a sharp sensitized maximum portion and a high red sensitivity.

The combined use of the sensitizing dyes according to this invention provides a silver halide emulsion having a higher red sensitivity compared to the use of each sensitizing dye alone and, at the same time, a very small inherent desensitization.

It is also possible to use at the same time another sensitizing dye for improving the green sensitivity (e.g., 2,2'-cyanine, thia-2'-cyanine etc.) or those having other spectral sensitizing wavelength regions.

The embodiments of sensitizing dyes used in this invention are mentioned as follows, but the sensitizing dyes used in this invention are not to be restricted only to those examples.





and



[II]



The carbocyanine dyes and sensitizing dyes of the general formula (II) which are used in this invention can be synthesized by a known method. For example, with reference to U.S. Pat. No. 2,503,776 and German Pat. Nos. 929,080 and 1,072,765, those skilled in the art can readily synthesize them.

The synthesis of a typical sensitizing dye of the general formula (I) is described as follows:

Synthesis — Dye C

One gram of 5-chloro-3-( $\gamma$ -sulfopropyl)-2-thiopropionyl-methylenebenzothiazoline is reacted with 1 g of methyl p-toluenesulfonate at 110° – 120° C for 2 hrs and then treated with ethyl ether to yield a methyl thiocarbinal compound. 1.1 g of 5-acetylaminomethyl-3-ethyl-2-methylbenzothiazolium p-toluenesulfonate salt are added thereto, and dissolved in 160 ml of etha-

nol, 2 ml of further triethylamine are added and the whole is heated for 3 hrs under reflux. After the completion of reaction, the solvent is distilled off and treated with ethyl ether and then with acetone to yield coarse crystals of Dye C. The coarse crystals are recrystallized from a mixed solvent of chloroform/ methanol to yield 550 mg of Dye C having a melting point above 310° C and a  $\lambda_{max}^{CH_3OH}$  of 559 nm. Other sensitizing dyes can be obtained by a similar method to the process as mentioned above.

The physical values of typical embodiments of said carbocyanine dyes according to this invention are as follows:

| Dyestuff No. | M.P. (°C) | $\lambda_{max}^{CH_3OH}$ (nm) |
|--------------|-----------|-------------------------------|
| I-A          | >300      | 566                           |
| I-B          | >300      | 554                           |
| I-C          | >300      | 559                           |
| I-D          | 276       | 565                           |
| I-E          | >300      | 560.5                         |
| I-F          | 282       | 562                           |
| I-G          | 296.5     | 562                           |
| I-H          | 231       | 567                           |
| I-I          | >300      | 558.5                         |

The sensitizing dyes of the general formula (I) are used, in general.

The spectral sensitizing process according to this invention is effective for the spectral sensitization of any silver halide photographic emulsions. And, it can sensitize sufficiently an emulsion containing a hydrophilic colloid other than gelatin, for example, agar collodion, water soluble cellulose derivatives, polyvinyl alcohol and other synthetic or natural hydrophilic polymers. For the photographic emulsion used in this invention, a mixed silver halide emulsion such as silver iodobromide, chloroiodobromide, and the like is suitable.

For the preparation of spectrally sensitized photographic emulsions according to this invention, it is enough to add the sensitizing dyes to a photographic emulsion in a common manner. In practice, it is convenient to add the dyes as a solution thereof in a suitable solvent such as methanol, ethanol, cellosolve etc., to the emulsion. The mol ratio of the sensitizing dyes according to this invention to be contained in the emulsion may be varied within a wide range of from 9:1 to 1:9 corresponding to the effect desired.

The photographic emulsion according to this invention may be treated by a known method for hyper- and

other super-sensitization. In the preparation of photographic emulsions according to this invention, additives which are generally used in the art of photographic emulsion manufacturing, for example, chemical sensitizers, stabilizers, toners, hardeners, wetting agents, anti-foggants, plasticizers, development accelerators, color developers and fluorescent brightening agents may be added further to the emulsion in a common manner.

10 The photographic emulsion according to this invention may be coated onto a suitable support, for example, glass plates, films of cellulose derivatives, films of synthetic resins, resin-laminated paper, or Baryta paper in a common manner.

The present invention will be illustrated further by reference to the following non-limiting examples.

## EXAMPLES

Sensitizing dyes used in this invention as mentioned 20 above were added individually to a silver iodobromide emulsion (AgI : AgBr = 7:93 in mol percent to prepare silver halide photographic emulsions. On the other hand, silver halide photographic emulsions containing a combination of the sensitizing dyes of this invention 25 were also prepared.

These emulsions were coated onto a cellulose triacetate film base, dried, exposed through a red filter (transmitting rays of a wavelength longer than 580 nm) and a blue filter (transmitting rays of a wavelength of 30 400 – 490 nm and having a maximum transmission at 450 nm) to a daylight of 64 Luxes (corresponding to 5,400° K) and developed.

As the developer, one having the following composition was used.

TABLE 1

|                |          |
|----------------|----------|
| Metol          | 2 g      |
| sodium sulfite | 100 g    |
| Hydroquinone   | 5 g      |
| Borax          | 2 g      |
| Water to make  | 1000 ml. |

The relative red sensitivity and inherent desensitization to the original emulsion for the single use of the sensitizing dyes as well as in the combined use of said sensitizing dyes according to this invention are shown 45 in the following Table 2.

TABLE 2

| Experimental No. | Example No. | Dye No. | Amount of sensitizing dye added (10 <sup>-5</sup> mol/kg emulsion) | Dye No. | Amount of sensitizing dye added (10 <sup>-5</sup> mol/kg emulsion) | Emulsion | Sensitized maximum wave length (nm) | Relative red sensitivity | Inherent sensitivity | Referred to in drawings |
|------------------|-------------|---------|--------------------------------------------------------------------|---------|--------------------------------------------------------------------|----------|-------------------------------------|--------------------------|----------------------|-------------------------|
| 1                | A           | A       | 4                                                                  |         |                                                                    | AgBr/I   | 656                                 | 125                      | 94                   | Fig. 3(8).              |
|                  |             | A       | 8                                                                  |         |                                                                    | AgBr/I   | 656                                 | 130                      | 85                   |                         |
|                  |             |         |                                                                    | 1       | 1                                                                  | AgBr/I   | 648                                 | 50                       | 90                   |                         |
|                  |             |         |                                                                    | 2       | 2                                                                  | AgBr/I   | 650                                 | 78                       | 90                   |                         |
|                  | 1           |         |                                                                    | 1       | 4                                                                  | AgBr/I   | 654                                 | 100                      | 90                   |                         |
|                  |             |         |                                                                    | 1       | 8                                                                  | AgBr/I   | 660                                 | 120                      | 85                   |                         |
|                  |             | A       | 4 1                                                                |         |                                                                    | 1 AgBr/I | 656                                 | 170                      | 94                   |                         |
|                  |             | A       | 4 1                                                                |         | 2                                                                  | AgBr/I   | 656                                 | 185                      | 94                   |                         |
| 2                | B           | B       | 2                                                                  |         |                                                                    | AgBr/I   | 600                                 | 5                        | 87                   | Fig. 3(7).              |
|                  |             | B       | 4                                                                  |         |                                                                    | AgBr/I   | 600                                 | 6                        | 80                   |                         |
|                  | 2 B         | 2       | 1                                                                  |         | 4                                                                  | AgBr/I   | 654                                 | 135                      | 90                   | Fig. 3(9).              |
|                  |             | C       | 2                                                                  |         |                                                                    | AgBr/I   | 648                                 | 100                      | 100                  |                         |
| 3                | C           | C       | 4                                                                  |         |                                                                    | AgBr/I   | 648                                 | 125                      | 187                  |                         |
|                  |             | C       | 8                                                                  |         |                                                                    | AgBr/I   | 648                                 | 140                      | 87                   |                         |
|                  | C           |         | 2                                                                  |         | 1                                                                  | AgBr/I   | 662                                 | 50                       | 93                   |                         |
|                  |             |         | 2                                                                  |         | 2                                                                  | AgBr/I   | 662                                 | 100                      | 90                   |                         |
| 3 C              | C           | 4 2     |                                                                    |         | 1                                                                  | AgBr/I   | 654                                 | 185                      | 94                   |                         |
|                  | C           | 4 2     |                                                                    |         | 2                                                                  | AgBr/I   | 656                                 | 190                      | 94                   |                         |

TABLE 2.—Continued

| Experimental No. | Example No. | Dye No. | Amount of sensitizing dye added (10 <sup>-5</sup> mol/kg emulsion) | Dye No. | Amount of sensitizing dye added (10 <sup>-5</sup> mol/kg emulsion) | Emulsion | Sensitized maximum wave length (nm) | Relative red sensitivity | Inherent sensitivity | Referred to in drawings |
|------------------|-------------|---------|--------------------------------------------------------------------|---------|--------------------------------------------------------------------|----------|-------------------------------------|--------------------------|----------------------|-------------------------|
| 4                |             | D       | 2                                                                  |         |                                                                    | AgBr/I   | 600                                 | 10                       | 90                   |                         |
|                  |             | D       | 4                                                                  |         |                                                                    | AgBr/I   | 634                                 | 13                       | 87                   |                         |
|                  |             | D       | 8                                                                  |         |                                                                    | AgBr/I   | 634                                 | 26                       | 87                   |                         |
| 5                | 4           | D       | 4                                                                  | 1       | 2                                                                  | AgBr/I   | 652                                 | 120                      | 96                   |                         |
|                  |             | D       | 4                                                                  | 1       | 4                                                                  | AgBr/I   | 660                                 | 135                      | 96                   |                         |
| 6                |             | E       | 4                                                                  |         |                                                                    | AgBr/I   | 600                                 | 16                       | 93                   | Fig. 2(4).              |
|                  |             | E       | 8                                                                  |         |                                                                    | AgBr/I   | 600                                 | 38                       | 93                   |                         |
|                  |             |         |                                                                    | 4       | 2                                                                  | AgBr/I   | 632                                 | 60                       | 85                   | Fig. 2(5).              |
| 7                | 5           | E       | 4                                                                  | 4       | 2                                                                  | AgBr/I   | 632                                 | 110                      | 93                   | Fig. 2(6).              |
|                  |             | F       | 1                                                                  |         |                                                                    | AgBr/I   | 640                                 | 20                       | 96                   |                         |
|                  |             | F       | 2                                                                  |         |                                                                    | AgBr/I   | 640                                 | 36                       | 90                   |                         |
|                  |             | F       | 4                                                                  |         |                                                                    | AgBr/I   | 640                                 | 36                       | 80                   |                         |
| 8                | 6           | F       | 5                                                                  |         | 4                                                                  | AgBr/I   | 660                                 | 110                      | 62                   |                         |
|                  |             | F       | 5                                                                  |         | 4                                                                  | AgBr/I   | 648                                 | 145                      | 90                   |                         |
|                  |             | G       | 4                                                                  |         |                                                                    | AgBr/I   | 642                                 | 145                      | 90                   |                         |
| 9                |             |         | 6                                                                  |         | 1                                                                  | AgBr/I   | 648                                 | 36                       | 94                   |                         |
|                  |             |         | 6                                                                  |         | 2                                                                  | AgBr/I   | 650                                 | 62                       | 94                   |                         |
|                  |             |         | 6                                                                  |         | 4                                                                  | AgBr/I   | 650                                 | 100                      | 94                   |                         |
| 10               | 7           | G       | 4                                                                  | 6       | 1                                                                  | AgBr/I   | 648                                 | 170                      | 94                   |                         |
|                  |             | G       | 4                                                                  | 6       | 2                                                                  | AgBr/I   | 650                                 | 180                      | 94                   |                         |
| 11               |             |         | 3                                                                  |         | 2                                                                  | AgBr/I   | 600                                 | 25                       | 92                   |                         |
|                  |             |         | 3                                                                  |         | 4                                                                  | AgBr/I   | 630                                 | 50                       | 90                   |                         |
|                  |             |         | 3                                                                  |         | 8                                                                  | AgBr/I   | 630                                 | 85                       | 85                   |                         |
|                  | 8           | G       | 4                                                                  | 3       | 2                                                                  | AgBr/I   | 650                                 | 175                      | 94                   |                         |
|                  |             | G       | 4                                                                  | 3       | 4                                                                  | AgBr/I   | 650                                 | 180                      | 94                   |                         |
| 12               |             | H       | 4                                                                  |         |                                                                    | AgBr/I   | 630                                 | 100                      | 90                   | Fig. 1(1).              |
|                  |             | H       | 8                                                                  |         |                                                                    | AgBr/I   | 640                                 | 150                      | 80                   |                         |
|                  |             |         | 7                                                                  |         | 0.5                                                                | AgBr/I   | 685                                 | 73                       | 96                   | Fig. 1(2).              |
|                  |             |         | 7                                                                  |         | 1                                                                  | AgBr/I   | 686                                 | 146                      | 96                   |                         |
|                  |             |         | 7                                                                  |         | 2                                                                  | AgBr/I   | 686                                 | 158                      | 87                   |                         |
| 13               | 9           | H       | 4                                                                  | 7       | 0.5                                                                | AgBr/I   | 680                                 | 120                      | 96                   | Fig. 1(3).              |
|                  |             | H       | 4                                                                  | 7       | 1                                                                  | AgBr/I   | 682                                 | 170                      | 96                   |                         |
| 14               |             |         | 8                                                                  |         | 0.5                                                                | AgBr/I   | 665                                 | 50                       | 100                  |                         |
|                  |             |         | 8                                                                  |         | 1                                                                  | AgBr/I   | 665                                 | 105                      | 100                  |                         |
|                  |             |         | 8                                                                  |         | 2                                                                  | AgBr/I   | 665                                 | 130                      | 95                   |                         |
|                  |             |         | 8                                                                  |         | 4                                                                  | AgBr/I   | 665                                 | 145                      | 86                   |                         |
|                  | 10          | H       | 4                                                                  | 8       | 1                                                                  | AgBr/I   | 660                                 | 160                      | 96                   |                         |
| 15               | 11          | I       | 1                                                                  |         |                                                                    | AgBr/I   | 646                                 | 85                       | 95                   | Fig. 4(10).             |
|                  |             | I       | 2                                                                  |         |                                                                    | AgBr/I   | 664                                 | 105                      | 95                   |                         |
|                  |             |         | 9                                                                  |         | 2                                                                  | AgBr/I   | 638                                 | 75                       | 80                   |                         |
|                  |             |         | 9                                                                  |         | 4                                                                  | AgBr/I   | 640                                 | 85                       | 70                   | Fig. 4(11).             |
|                  |             |         | 9                                                                  |         | 8                                                                  | AgBr/I   | 640                                 | 85                       | 60                   |                         |
| 16               | 11          | I       | 1                                                                  | 9       | 4                                                                  | AgBr/I   | 642                                 | 130                      | 100                  | Fig. 4(12).             |
|                  |             | I       | 2                                                                  | 9       | 4                                                                  | AgBr/I   | 642                                 | 160                      | 96                   |                         |
|                  |             |         | 10                                                                 |         | 1                                                                  | AgBr/I   | 680                                 | 35                       | 90                   |                         |
| 17               | 12          | C       | 4                                                                  | 10      | 2                                                                  | AgBr/I   | 680                                 | 70                       | 85                   |                         |
|                  |             | C       | 4                                                                  | 10      | 4                                                                  | AgBr/I   | 680                                 | 120                      | 70                   |                         |
| 18               | 13          | 1       | 2                                                                  | 9       | 4                                                                  | AgBr/I   | 640                                 | 180                      | 106                  |                         |
| 19               | 14          | C       | 4                                                                  | 2       | 1                                                                  | AgBr/I   | 652                                 | 195                      | 100                  |                         |
| 20               |             |         | 11                                                                 |         | 2                                                                  | AgBr/I   | 652                                 | 20                       | 94                   |                         |
|                  |             |         | 11                                                                 |         | 4                                                                  | AgBr/I   | 654                                 | 90                       | 92                   |                         |
|                  |             |         | 11                                                                 |         | 6                                                                  | AgBr/I   | 658                                 | 130                      | 92                   |                         |
| 21               | 15          | G       | 4                                                                  | 11      | 2                                                                  | AgBr/I   | 652                                 | 175                      | 94                   |                         |
|                  |             | G       | 4                                                                  | 11      | 4                                                                  | AgBr/I   | 658                                 | 175                      | 94                   |                         |
|                  |             |         | 12                                                                 |         | 2                                                                  | AgBr/I   | 600                                 | 20                       | 92                   |                         |
| 22               |             |         | 12                                                                 |         | 4                                                                  | AgBr/I   | 626                                 | 48                       | 90                   |                         |
|                  |             |         | 12                                                                 |         | 8                                                                  | AgBr/I   | 626                                 | 75                       | 85                   |                         |
|                  | 16          | C       | 4                                                                  | 12      | 2                                                                  | AgBr/I   | 646                                 | 150                      | 94                   |                         |
|                  |             | C       | 4                                                                  | 12      | 4                                                                  | AgBr/I   | 646                                 | 165                      | 92                   |                         |

The red sensitivity is shown as a relative sensitivity assuming that the red sensitivity of sensitizing dye 1, exposed through a red filter (a filter transmitting rays of a wavelength longer than 580 nm) in an amount of 4  $\times 10^{-5}$  mol/kg emulsion is 100; and the inherent sensi-

tivity is shown as a relative sensitivity assuming that the sensitivity of the original emulsion which is exposed through a blue filter (a filter transmitting rays of from 400 to 490 nm and having a maximum transmission at 450 nm) is 100.

As is obvious from Table 2, the addition of a single sensitizing dye according to this invention reduces inherent sensitivity together with an increase of red sensitivity as the amount of dye added is increased. However, it is seen that the combined use of the sensitizing dyes provides a higher red sensitivity than in the single use of the corresponding sensitizing dye alone. As is also obvious from examples 13 and 14 in Table 2, the effect of the combination of said sensitizing dyes is not injured by the further addition of a green sensitizing dye thereto, e.g. the combined use of green sensitizing dye (i) or (ii) with the combination of the sensitizing dyes according to this invention.

The said green sensitizing dyes have the following chemical structures, but they are not restricted only to these sensitizing dyes.

Dye I



Dye II



What is claimed is:

1. A silver halide photographic emulsion containing a supersensitizing combination of at least one carbocyanine dye having two heterocyclic nuclei each of said nuclei comprising a benzothiazole or benzoselenazole nucleus, at least one of the heterocyclic nuclei having an acetylamino group at the 5-position thereof, and having a sensitized maximum portion within the range of from 600 to 660 nm, and at least one sensitizing dye of the following general formula (II)



wherein  $R_3$  and  $R_4$  each represents a lower alkyl group;  $A_2$  represents a lower alkyl group or an aryl group;  $Z_3$  and  $Z_4$  each represents an atomic group necessary to complete a benzothiazole, benzoselenazole or  $\beta$ -naphthothiazole nucleus;  $X_2^-$  represents an anion; and  $m$  is 0 or 1,  $m$  being 0 when an intermolecular salt is formed.

2. The silver halide photographic emulsion of claim 1 wherein the carbocyanine dye is represented by the following general formula (I) :



wherein  $R_1$  and  $R_2$  each represents a lower alkyl group;  $A_1$  represents a lower alkyl group;  $Z_1$  represents an

atomic group necessary to complete a benzothiazole or benzoselenazole nucleus;  $Z_2$  represents a sulfur or a selenium atom;  $X_1^-$  represents an anion, and  $n$  is 0 or 1,  $n$ , being 0 when an intermolecular salt is formed.

3. The silver halide photographic emulsion of claim 1 further containing at least one green sensitizing cyanine dye selected from the group consisting of 2,2'-cyanine and thia-2'-cyanine.

4. The silver halide photographic emulsion of claim 10 1 wherein said carbocyanine dye is selected from the group consisting of

[I]

Dye A



Dye B



Dye C



Dye D



Dye E



Dye F



Dye G



Dye H



and



5. The silver halide photographic emulsion of claim 1, wherein said sensitizing dye is selected from the group consisting of



\* \* \* \*